

## UNITED STATES PATENT OFFICE

2,209,976

## STABILIZED OIL COMPOSITION

William H. James, Paulsboro, N. J., assignor to  
Socony-Vacuum Oil Company, Incorporated,  
New York, N. Y., a corporation of New York

No Drawing. Application January 20, 1938,  
Serial No. 185,907

12 Claims. (Cl. 252—47)

This invention has to do in a general way with hydrocarbon oil compositions and is more particularly related to refined viscous petroleum oils which have been stabilized against the deteriorating effects of oxidation by the incorporation therein of a small amount of an antioxidant or oxidation inhibitor.

As is well known to those familiar with the art, refined viscous petroleum oil fractions, such as transformer oils, turbine oils, motor oils, and the like, which have been refined by treatment with sulfuric acid or by other methods such as by solvent refining, are prone to deterioration, due to the effects of oxidation reactions, under the normal conditions of use at elevated temperatures, particularly when in contact with metals. This oxidation results in the formation of acidic products which decrease the insulating or dielectric strength of the oil, thereby diminishing its usefulness in such applications as transformers and the like, and which are corrosive in nature and thereby decrease the usefulness of the oils for lubrication.

This invention has as its object the provision of refined viscous petroleum oils which are substantially stable against oxidation under normal conditions of use and of a method of protecting such oils against oxidation.

My invention is based upon the discovery of the fact that materials obtained as the reaction product of an alkylamine and a chloride of sulfur, when blended with refined viscous petroleum oils of the types above referred to, will substantially stabilize such oils against the deteriorating effects of oxidation.

The oil stabilizing compounds contemplated by this invention, which may, for the purpose of identification, be termed *N,N'-thio-bis-alkylamines*, are characterized by the fact that they contain sulfur linked at least by one valence bond to nitrogen. These compounds are obtained as indicated above by the interaction of sulfur chlorides, such as sulfur monochloride, sulfur dichloride, etc., with primary or secondary alkylamines. Compounds of this character perform the function of oxidation and corrosion inhibitors when blended with refined viscous petroleum oils of the type above referred to in amounts less than 0.1%.

As indicated above, the field of my invention is not restricted to the so-called "highly refined" oil of the character of transformer oils and turbine oils, but also includes solvent refined motor oils. In this latter regard, it is well known to those familiar with the art that solvent refining

of mineral oil has made possible the marketing of motor oils of higher viscosity index than heretofore has been available, but that these solvent refined oils of high viscosity index have a decided tendency to corrode hard bearings, such as the cadmium-silver alloy type of bearings. The compounds contemplated by this invention as corrosion inhibitors I have found to be particularly valuable as additive ingredients for solvent refined oils to inhibit the corrosive action of such oils on bearing materials of this character, and it is therefore a further object of this invention to provide a method for protecting alloy bearings, such as cadmium-silver bearings, from the corrosive action of solvent refined motor oils by maintaining within the lubricating film between the bearing surfaces a compound of the type described.

As has been previously stated, the *N,N'-dithio-bis-dialkylamines* contemplated by this invention can be obtained by the reaction of a sulfur chloride on a dialkylamine. To illustrate the method of synthesizing these compounds the following example is given: 4 moles (628 grams) of diethylamine was added to 800 cc. of benzene in a reaction vessel. One mole (135 grams) of sulfur monochloride diluted with 200 cc. of benzene was then gradually added to the amine solution. It was necessary to employ two equivalents of amine, since two moles of the amine were consumed in the formation of a hydrochloride salt which was apparently unreactive with the sulfur monochloride. After the sulfur monochloride had been added, the mixture was cooled and stirred until the heat of reaction had been dissipated; the amine hydrochloride was filtered off and the benzene removed from the filtrate by distillation. Any unreacted diethylamine was removed by distilling under reduced pressure. The final product may be water-washed if desired, but it was found to be equally effective as a corrosion inhibitor whether washed or not.

*N,N'-dithio-bis-dibutylamine* and *N,N'-dithio-bis-dicyclohexylamine* were also prepared according to this method by the action of sulfur monochloride on dibutylamine and dicyclohexylamine respectively.

The reaction which probably takes place in the synthesis described above may be represented by the following general equation:



in which R and R' may both represent alkyl groups or in which R may represent an alkyl

group and R' may represent hydrogen, and in which x represents the numeral 1 or 2. For the reaction with diamylamine given in the example above this reaction may be represented as follows:



The N, N'-dithio-bis-alkylamines contemplated by this invention have the probable general formula



- 15 in which R and R' both represent alkyl groups, in the case of a N,N'-dithio-bis-dialkylamine, or in which R represents an alkyl group and R' represents hydrogen, in the case of a N,N'-dithio-bis-monoalkylamine.
- 20 As stated above, the compounds contemplated by this invention are particularly useful in the stabilization of motor oils. To demonstrate this, the following test was performed with a solvent refined motor oil having a Saybolt Universal viscosity of 55 seconds at 210° F. and a flash point of 435° F. The test comprised bubbling air through a 30 gram sample of oil, heated to 347° F. at the rate of 2,000 ml. per hour over a period of 22 hours, in the presence of a piece of cadmium-silver alloy bearing. The following table shows the loss in weight in milligrams of the piece of test metal, using the mineral oil alone and the same oil inhibited with N,N'-dithio-bis-diamylamine, N,N'-dithio-bis-dibutylamine and 35 N,N'-dithio-bis-dicyclohexylamine, or more specifically, with the products obtained by the reaction of diamylamine, dibutylamine, and dicyclohexylamine with sulfur monochloride according to the exemplary synthesis given above:

40

Table I

| 45 | Compound                          | Percent<br>in oil | Loss in weight of<br>bearing, milli-<br>grams |                  |
|----|-----------------------------------|-------------------|-----------------------------------------------|------------------|
|    |                                   |                   | Oil<br>alone                                  | Inhibited<br>oil |
|    | N,N'-dithio-bis-dibutylamine      | 0.10              | 40                                            | 0                |
|    | N,N'-dithio-bis-diamylamine       | 0.10              | 75                                            | 0                |
| 50 | Do                                | 0.05              | 75                                            | 0                |
|    | Do                                | 0.01              | 58                                            | 2                |
|    | N,N'-dithio-bis-dicyclohexylamine | 0.25              | 40                                            | 0                |
|    | Do                                | 0.10              | 67                                            | 0                |

In addition to the N,N'-dithio-bis-dialkylamines I have also prepared representative compounds of the N,N'-dithio-bis-monoalkylamine type in which the primary amines mono-butylamine and mono-cyclohexylamine were used as the reactants. These compounds, N,N'-dithio-bis-monobutylamine and N,N'-dithio-bis-mono-cyclohexylamine, although only slightly soluble in oil were found to be effective as corrosion inhibitors in the bubble test described above, as indicated by the data in Table II below:

65

Table II

| 70 | Compound                            | Percent<br>in oil | Loss in weight of<br>bearing, milli-<br>grams |                  |
|----|-------------------------------------|-------------------|-----------------------------------------------|------------------|
|    |                                     |                   | Oil<br>alone                                  | Inhibited<br>oil |
|    | N,N'-dithio-bis-monobutylamine      | <0.25             | 110                                           | 1                |
|    | N,N'-dithio-bis-monocyclohexylamine | 0.25              | 40                                            | 1                |

75

To illustrate the effectiveness of the compounds contemplated by this invention as means for inhibiting the formation of acidic oxidation products in highly refined oils such as transformer oils and the like, the following test was performed. A neutral transformer oil with Saybolt Universal viscosity of 70 seconds at 100° F. was heated in a glass container for 70 hours at a temperature of 250° F. in the presence of oxygen. At the end of this period the acidic value or 10 neutralization number (N. N.) of the oil was determined. The test was repeated with a sample of the same oil containing various N,N'-dithio-bis-dialkylamines, and the results of this test, which is known as the Modified German tar 15 test, are given in the table below:

Table III

|                                                  | N. N. after aging | 25.0 |
|--------------------------------------------------|-------------------|------|
| Oil alone                                        |                   | 20   |
| Oil+0.10% N,N'-dithio-bis-dibutylamine           | 0.06              | 11   |
| Oil+0.10% N,N'-dithio-bis-diamylamine            | 0.11              |      |
| Oil+0.10% N,N'-dithio-bis-dicyclohexyl-<br>amine | 0.06              |      |

It will be seen from the above data that the 25 compounds contemplated by this invention, which are represented by the reaction products of dialkylamines and monoalkylamines with sulfur monochloride, possess a high degree of capability of inhibiting the oxidation and corrosion effects of highly refined or solvent refined mineral oils. It will be observed that the percentage of the inhibitive compound required is very low, substantial inhibition being obtained with the use of as little as from 0.01% to 0.25% of the ingredients.

I claim:

1. A mineral oil composition comprising a refined viscous mineral oil having incorporated therein a small amount sufficient to stabilize the oil against the deteriorating effects of oxidation of a N,N'-dithio-bis-alkylamine.
2. A mineral oil composition comprising a refined viscous mineral oil having incorporated therein a small amount sufficient to stabilize the oil against the deteriorating effects of oxidation of a N,N'-dithio-bis-dialkylamine.
3. A mineral oil composition comprising a refined viscous mineral oil having incorporated therein a small amount sufficient to stabilize the oil against the deteriorating effects of oxidation of a N,N'-dithio-bis-monoalkylamine.
4. A mineral oil composition comprising a refined viscous mineral oil having incorporated therein a minor proportion sufficient to stabilize the oil against the deteriorating effects of oxidation of a compound selected from the group consisting of: N,N'-dithio-bis-dibutylamine; N,N'-dithio-bis-diamylamine; N,N'-dithio-bis-dicyclohexylamine; N,N'-dithio-bis-monobutylamine; and N,N'-dithio-bis-monocyclohexylamine.
5. A mineral oil composition comprising a refined viscous mineral oil having incorporated therein a minor proportion sufficient to stabilize the oil against the deteriorating effects of oxidation of N,N'-dithio-bis-diamylamine.
6. A mineral oil composition comprising a refined viscous mineral oil having incorporated therein a minor proportion sufficient to stabilize the oil against the deteriorating effects of oxidation of N,N'-dithio-bis-dibutylamine.
7. A mineral oil composition comprising a refined viscous mineral oil having incorporated therein a minor proportion sufficient to stabilize

the oil against the deteriorating effects of oxidation of N,N'-dithio-bis-dicyclohexylamine.

8. A mineral oil composition comprising a refined viscous mineral oil having incorporated therein a minor proportion sufficient to stabilize the oil against the deteriorating effects of oxidation of a compound having the probable formula



in which R and R' represent alkyl groups.

9. A mineral oil composition comprising a refined viscous mineral oil having incorporated therein a minor proportion sufficient to stabilize the oil against the deteriorating effects of oxidation of a compound having the probable formula



in which the R's represent alkyl groups and in which the R's represent radicals selected from

the group consisting of hydrogen and alkyl groups.

10. A mineral oil composition comprising a refined viscous mineral oil having incorporated therein a small amount of N,N'-thio-bis-alkyl- 5 amine.

11. A mineral oil composition comprising a refined viscous mineral oil fraction having incorporated therein from about 0.01 per cent to about 0.25 per cent of an N,N'-dithio-bis-alkylamine. 10

12. A mineral oil composition comprising a refined viscous mineral oil having incorporated therein a minor proportion of from about 0.01 per cent to about 0.25 per cent of a compound having the general formula 15



in which the R's represent alkyl groups and in which the R's represent radicals selected from the group consisting of hydrogen and alkyl groups. 20

WILLIAM H. JAMES.